

## UNITED STATES PATENT OFFICE

2,151,641

## GREASE BASE AND METHOD OF MAKING

Latimer D. Myers, Cincinnati, Ohio, assignor to  
Emery Industries, Inc., Cincinnati, Ohio, a cor-  
poration of Ohio

No Drawing. Application December 21, 1936,  
Serial No. 116,996

9 Claims. (CL 87—9)

This invention relates to the preparation of bases particularly adapted to be used in the manufacture of lubricating greases. The invention comprehends a new series of grease bases, or substances adapted to use in the preparation of greases from mineral oils, and comprehends also a new method by means of which these bases are prepared.

In the past it has been conventional to manufacture greases from mineral oil, soap and water. In the more or less conventional types of greases adapted to use for general lubricating purposes, the calcium soaps have been used quite extensively. Greases of this nature essentially comprise emulsions of oil and water in which the water is held in the oil by the action of the soap.

More recently, it has been determined that the greases which are in anhydrous condition possess qualities which are not possessed by the greases of the moisture variety. The greases which contain moisture essentially comprise emulsion of water in oil, in which the soap is present to maintain the emulsion in the established state. In these greases the tendency is for the emulsion to break and the oil to separate during periods of storage or long standing. The body and consistency of these greases permanently is lost if or when the greases are subjected to temperatures sufficiently high to drive off any substantial quantity of the water which is present.

The anhydrous greases on the other hand are not dependent upon the presence of water for their stability, but to the contrary, the less water they contain, the more efficiently they seem to function. The primary objective of the present invention has been to provide a series of bodies which are dry and which are particularly adapted to be used in making greases which are dry.

By reason of the fact that the present invention provides a series of anhydrous bases, comprised of metal soaps of fatty acids, which are very much superior to the soaps which heretofore have been available and which possess the capacity to make better greases than those which have been available, a brief analysis of various methods for making the metallic soaps of fatty acids is requisite to the full understanding of the present advance.

In the past it has been conventional to prepare the soaps used for making greases of the calcium soap variety by the double decomposition of a water soluble soap, for example, a sodium soap with a water soluble calcium salt, in aqueous solution. Usually, sodium soaps are first pre-

pared in the ordinary manner, then these soaps are dissolved in water, and finally the calcium salt (for example, calcium chloride) gradually is added to the solution to cause precipitation of insoluble calcium soap, which then is filtered off or separated from the remaining liquid in any convenient manner. This soap next is washed free of inorganic salts and finally is dried. The process obviously is expensive; it requires extensive equipment; and a proportionately large quantity of sodium chloride, which has little or no value, is left as a by-product or waste.

Another method of preparing the calcium soaps of fatty acids involves the saponification of fats with lime. While this process in general is less expensive than the method of double decomposition, still, pressure is required during the saponifying procedure, the saponification is relatively difficult to conduct and still more difficult to complete and the final product is not in an anhydrous state.

Still another process for preparing calcium soaps of fatty acids is predicated on the fusion of fatty acids with lime. According to this process, the fatty acids are melted and fusion with the lime takes place at relatively high temperature. During the reaction, a heavy molten mass develops. The difficulty is that as the reaction continues, and as the fatty acid content in the admixture is reduced, this mass becomes less molten and more viscous. Thorough stirring and mixing becomes difficult, and some of the material in the vessel sticks to the sides of the container and tends to become charred or otherwise badly discolored. The process as a whole is not well suited to commercial production methods.

The pure dry fatty acid soaps of calcium, zinc, magnesium, and the like can be made to dissolve in mineral oil at elevated temperature. On the other hand, at ordinary room temperatures these same soaps are almost totally insoluble. If solutions of the soaps are made in oil at high temperature and are allowed to cool and set to gels, the difficulty is that these gels are broken easily by stirring or other mechanical disruption, and, when this occurs, the body of the grease is lost and the soaps precipitate.

In my copending patent application Serial No. 952, I have disclosed a process for preparing anhydrous greases which are stable and which are strong in lattice structure. According to this process an auxiliary material is used which effects dissolution of the soap in the oil at ordinary temperature. I have disclosed in this copending

application that the compounds of high molecular weight containing free hydroxyl groups and particularly the esters formed by partial esterification of polyhydric and dihydric alcohols with higher fatty acids, are well suited to the purpose.

The grease bases of the present invention are anhydrous products which are characterized by their solubility in mineral oil at relatively low temperature, next by the presence of a quota of a metallic soap of a fatty acid, and furthermore by the presence of a quota of a substance containing free hydroxyl groups adapted to effect dissolution of the soap of the base in mineral oils at ordinary temperatures. The provision of bases for making greases which are thus characterized, and a process by means of which these bases are obtained comprise the primary objectives of the invention.

Briefly, the concept or the principle upon which the present invention is predicated resides in a process in which two reactions are caused to take place substantially conjointly. In the first of these reactions a quantity of metallic soap of fatty acid is formed by the fusion method but the quantity of fatty acid which is present during the fusion is in excess of that required to make the soap. In the other reaction this excess or free quantity of fatty acid is changed in situ to a fatty acid derivative which is soluble in mineral oil; which is relatively nonvolatile and which has a solvent action or tendency in relation to the fatty acid soap.

According to my copending patent application previously identified, I have disclosed that typical compounds having free hydroxyl groups suitable for the purpose of effecting dissolution of the calcium soap in the mineral oil under the conditions preferred, are the partial esters of fatty acids such as stearic, and the polyhydric or dihydric alcohols. These esters commonly are prepared by heating to a relatively high temperature (around 250° C.) a mixture of polyhydric or dihydric alcohol and fatty acids. Esterification occurs relatively slowly. Several hours are required to effect the combination, and the operation usually must be carried out under a vacuum, or in the atmosphere of an inert gas, in order to prevent excessive discoloration of the final products. Likewise, it previously has been pointed out that the fusion or reaction of a dry metal salt with fatty acid is difficult to conduct because of the problems encountered in stirring and handling the mass which becomes more and more viscous as the reaction proceeds to completion.

Paradoxically, however, it is the concept of the present invention to combine two reactions, each slow and difficult to conduct individually, and provide a process for making the products desired, which is conducted with much more ease and with much greater convenience than in either process and which proceeds to completion much more rapidly. Thus, a conjoint reaction is established, and the desired anhydrous condition of the base is accomplished.

In the practice of the present invention, the use of a quota of fatty acid in excess of that required to produce the metallic soap has two-fold significance. In the first place, if the quantity of fatty acid is in the right amount to combine with the alkali to make the soap then as the reaction proceeds, the mixture becomes very difficult to handle. The excess of fatty acid, however, in a sense has the function of a diluent or solvent. When this excess is present it thins down the mixture at the time that the soap is being formed

and consequently the difficulties in stirring and handling are obviated.

On the other hand the excess provides a quota of fatty acid from which to derive a substance which renders the metallic soap soluble in mineral oil and which also acts as a solvent for the metallic soaps with the result that the mix remains relatively fluid at all stages of the operation. Thus, the process is characterized by two features. The consistency of the mass is relatively thin and workable even as the free fatty acid content is lowered by the formation of soap, and the agent for stabilizing the soap and effecting its dissolution in mineral oil at room temperature is provided in the mass with ease and convenience.

The present invention particularly is disclosed in relation to the formation of the partial esters of the polyhydric and dihydric alcohol and fatty acids as the bodies adapted particularly to effect the dissolution and stabilization of the metallic soap in mineral oil. The disclosure of these bodies is representative of a preferred embodiment which is specific to the generic principle which is involved.

The following examples illustrate the procedure for making various grease bases in accordance with the present invention:

*Example 1—Lime soap base in which glyceryl mono stearate is present—*

The optimum proportion of calcium stearate and glyceryl mono stearate for any given oil which is to be used for the manufacture of a grease is determined empirically before hand, that is by making greases and determining the mixture which yields the most desirable product. The fatty acid, which preferably is stearic acid, is then introduced into a suitable container either direct-fired or steam-jacketed and heated to about 110° C. Next, the requisite quantity of dry powdered lime is added slowly. Reaction occurs very readily and the mass remains fluid due to the presence of the excess of fatty acid.

The quantity of polyhydric alcohol required to combine with the remaining fatty acid is added, mole for mole, preferably after a short period of time with continued heating, the temperature being raised to 180° C. The reaction proceeds smoothly and the mass remains fluid as the hydroxy ester which is formed is also a solvent for the soap produced in the prior step. After about two hours the free fatty acid usually is less than 5% and the resulting product is poured into molds to solidify or may be poured over a flaking roll.

The peculiar thing which will be noted is that the metallic soap which is formed seems to catalyze the reaction between the excess of fatty acid and the alcohol. Ordinarily, it is relatively difficult to accomplish partial esterification in a relatively reasonable time. Still, in the presence of the fatty acid soap esterification proceeds relatively rapidly. And as the excess of fatty acid is esterified the fluidity, or workability of the mass as a whole does not change appreciably in view of the fact that the fatty acid esters at the reaction temperature themselves are in relatively fluid condition. This aspect of the invention is, of course, of great commercial importance so far as the industrial production of these bodies is concerned.

The final temperature (180°) is considerably lower than that required to complete the production of the hydroxy ester when no calcium soap is present, particularly in view of the fact that the theoretical quantity, or only very slightly over

the theoretical quantity of higher fatty alcohol is employed. At the same time the fatty acid esters which are formed maintain the calcium soaps in fluid condition.

5 *Example 2—Preparation of a base consisting of four parts calcium stearate and one part glyceryl mono stearate—*

1140 parts of stearic acid are heated to 130° C. and 128 parts of powdered lime added slowly over a period of about fifteen minutes. After an additional fifteen minutes the free fatty acid of the mix will be about 29%. 68 parts of glycerine are then added and the temperature raised to 130° C. It has been my experience that after one hour (total time) the free fatty acid will have decreased to 7.3%, after 1½ hours to 5.2% and after two hours to 4%. Next, agitation is increased and the temperature is allowed to drop somewhat during the last few minutes of the run. This incorporates air in the product, which finally is moulded. The entrained air renders the product friable and easily powdered.

25 Other proportions of calcium stearate and glyceryl mono stearate are prepared by the use of the proper amounts of lime and glycerine. A ratio of six parts of calcium stearate to one part of glyceryl mono stearate is about the maximum which can be prepared conveniently as this mixture contains about the minimum quantity of mono stearate which is capable of keeping the fused mass in a relatively fluid state.

35 In the practice of the invention, it is preferred to saponify the fatty acid with one of the usual calcium salts, such as lime, in order to provide the corresponding calcium soap. However, the process of the invention is adapted to use in the production of bases for making greases in which other soaps than the calcium soaps are used. Thus, the salts appropriate to the production of 40 magnesium, zinc, lead, cobalt, and similar soaps of high titre fatty acids such as stearic or palmitic may be used as substitutes for the calcium salts.

45 Other substances likewise can be used in place of the glycerine to react with the excess of fatty acid to provide fatty acid esters thereof mingled with fatty acid soap.

50 In general, it is the concept of the invention to esterify this excess of fatty acid to a substance which has the general formula A—OH in which OH represents a hydroxyl group and in which A is an organic radical of such nature that the A—OH compound is soluble in mineral oil, relatively nonvolatile and has a soluble action or 55 tendency in relation to fatty acid soap.

55 The A—OH compound preferably consists of a partial ester of a polyhydric or dihydric alcohol and a fatty acid. Examples of substances which may be used in place of glycerine to produce this 60 compound are ethylene glycol, diethylene glycol, propylene glycol and the like.

65 *Example 3—To prepare a grease base consisting of 4 parts of calcium stearate and one part of diethylene glycol monostearate, about—*

65 720 parts of stearic acid are melted and heated to approximately 160° C. and about 32 parts of hydrated lime added slowly over a period of about one-half an hour to prevent lumping. When 70 practically all of the lime has reacted, which may require from ½ to 1 hour depending upon the degree and type of agitation, about 18 parts of diethylene glycol is added and the temperature raised to 160° C. The heating is continued until 75 the free fatty acid content has dropped to below

10%. If the heating is carried out in an open vessel additional diethylene glycol may be required to compensate for loss by evaporation.

Free fatty acid tests on the material as the reaction proceeds show 30.9% free fatty acid after 5 the lime is added, 16.5% after ½ hour heating, 14.4% after one hour heating and 13.5% after 1½ hours. The addition of 9 parts of diethylene glycol to compensate for evaporation followed by ½ hour heating gives a final free fatty acid of 6%. 10

The reaction product is a syrupy mass when hot and upon cooling forms a tan-colored hard waxy mass.

7.5% of this product dissolved in 200 sec. mineral oil produces a clear transparent water-free 15 grease.

Example 4—*To prepare a grease base consisting of 4 parts of calcium stearate and one part of ethylene glycol stearate, about—*

20 276 parts of stearic acid  
32 parts of calcium hydroxide, and  
121 parts of ethylene glycol  
are processed as described in Example 3. The reaction progresses about as shown by free fatty 25 acid determinations as follows:

|                                           |    |         |
|-------------------------------------------|----|---------|
| After lime added FFA                      | —  | %— 29.5 |
| ½ hour heating                            | —  | 14.7    |
| 1½ hour heating                           | —  | 12.2    |
| 6 parts additional glycol 1½ hrs. heating | %— | 7.6 30  |

The product has substantially the same appearance as that described in Example 3. 7.5 parts of this base dissolved in 200 sec. mineral oil gives a clear anhydrous grease considerably 35 heavier than that produced by the product of Example 3.

Example 5—*Preparation of a grease base consisting of 2 parts of sodium stearate and one part of diethylene glycol monostearate, about—*

40 253 parts of stearic acid  
20.6 parts sodium hydroxide dissolved in the minimum quantity of water  
45.2 parts of diethylene glycol

45 are treated in the manner disclosed in Examples 3 and 4. The final free fatty acid content is about 11.5%.

This base is softer than the calcium soap bases and has more of the ordinary soap-like feel. It 50 is not suitable by itself for preparing a grease but can be added to oil in small proportions along with the grease bases already described to impart a stringy characteristic to the greases.

The grease bases which are made in accordance with the process of the present invention are 55 anhydrous or substantially so. Small quantities of water may be included in them without necessarily destroying their value or their utility. Of course, it is recommended that the bases be used 60 in a condition as nearly anhydrous as possible for the reason that the greases which they themselves are adapted to provide are in general of improved appearance and superior stability, more uniform in consistency and more easily manufactured to precise specifications.

65 In making greases from the grease bases which I have provided, it is necessary only to dissolve the base in the requisite quantity of oil, then cool this mixture either by pouring it into containers 70 or by passing it over a chilling roll. It is recommended that the grease base be dissolved completely in the oil before the mixture is chilled, to form the grease. If desired, the oil can be heated 75 to a temperature of around 150°, more or less,

to increase the rate of dissolution. The greases which are made from the grease bases of the present invention are anhydrous or substantially so. The grease base component, when once dissolved in the mineral oil, does not tend to precipitate from the grease as in the greases of the moisture variety, and therefore, these greases are particularly well adapted to use for lubricating purposes, under relatively high temperature conditions.

Having described my invention, I claim:

1. A method of making a body which is soluble in mineral oil at room temperature which method comprises, conjointly fusing fatty acid with calcium oxide lesser in amount than that required to react with the fatty acid to make a soap, and esterifying the balance of the fatty acid with an aliphatic polyhydric alcohol, to produce a fatty acid ester having at least one free hydroxyl group.

2. The method of making a grease base which is substantially anhydrous, which method comprises, reacting a fatty acid with a calcium salt, reactive with fatty acid to form a soap, but insufficient in amount to react with all of the fatty acid, then reacting, in situ, the uncombined fatty acid with a high boiling alcohol, whereby to provide a mass comprised of calcium salt of fatty acid mingled with a fatty acid ester having at least one free hydroxyl group.

3. The method which consists in substantially conjointly reacting a fatty acid with lime, insufficient in amount to react with all of the fatty acid, and with a high boiling alcohol adapted to esterify the remainder of the fatty acid, to provide a body consisting of the calcium salt of fatty acid mingled with a fatty acid ester having at least one free hydroxyl group.

4. The method which comprises, reacting lime with a quota of stearic acid in excess of the quota required to combine with the lime, then reacting the excess of fatty acid with a high boiling alcohol to provide, in the presence of the calcium salt of fatty acid, a fatty acid ester having free hydroxyl groups.

5. The method of making a base soluble in mineral oil to provide an anhydrous grease there-

from, which method comprises, forming a dry soap of a fatty acid in the presence of a quantity of fatty acid in excess of that required to form the soap and reacting the excess of fatty acid with an aliphatic alcohol which is reactive in respect thereto to form, in situ, a fatty acid ester having at least one free hydroxyl group.

6. A method of making a grease base which comprises, heating a mass of fatty acid partially saponified with lime with a polyhydric alcohol to esterify the saponified component of the fatty acid, to provide in the mass a quota of fatty acid ester having at least one free hydroxyl group, which is soluble in mineral oil and which possesses the capacity to dissolve the fatty acid component which is saponified.

7. The method of making an anhydrous grease base which comprises, forming a mass containing free fatty acid and fatty acid soap adapted to make a grease with mineral oil, and heating this mass with a quota of material reactive in respect to the free fatty acid, to provide a reaction component in the mass which has at least one free hydroxyl group and which is soluble in mineral oil and which is a solvent for the fatty acid soap.

8. A method of making an anhydrous grease base which consists in forming a fatty acid soap adapted to make a grease with mineral oil, and forming a partial ester of fatty acid which has at least one free hydroxyl group, in situ, during at least a portion of the time that the soap is being formed, the amount of ester formed being sufficient to solubilize the soap in mineral oil sufficient in quantity to make a grease therewith.

9. The method of making an anhydrous body soluble in mineral oil to form a grease therefrom, which method consists in saponifying a major portion of a body of fatty acid to form a substantially anhydrous fatty acid soap and in reacting the remaining minor portion of fatty acid with a body adapted to provide therefrom a reaction component which has at least one free hydroxyl group, which is soluble in mineral oil, which is a solvent for fatty acid soap and which is present in sufficient quantity to render all of the said soap soluble in mineral oil.

LATIMER D. MYERS.

#### CERTIFICATE OF CORRECTION.

Patent No. 2,151,641.

March 21, 1939.

LATIMER D. MYERS.

It is hereby certified that error appears in the printed specification of the above numbered patent requiring correction as follows: Page 3, second column, line 10, for "6%" read 6.9%; and that the said Letters Patent should be read with this correction therein that the same may conform to the record of the case in the Patent Office.

Signed and sealed this 18th day of April, A. D. 1939.

Henry Van Arsdale

(Seal)

Acting Commissioner of Patents

to increase the rate of dissolution. The greases which are made from the grease bases of the present invention are anhydrous or substantially so. The grease base component, when once dissolved in the mineral oil, does not tend to precipitate from the grease as in the greases of the moisture variety, and therefore, these greases are particularly well adapted to use for lubricating purposes, under relatively high temperature conditions.

Having described my invention, I claim:

1. A method of making a body which is soluble in mineral oil at room temperature which method comprises, conjointly fusing fatty acid with calcium oxide lesser in amount than that required to react with the fatty acid to make a soap, and esterifying the balance of the fatty acid with an aliphatic polyhydric alcohol, to produce a fatty acid ester having at least one free hydroxyl group.

2. The method of making a grease base which is substantially anhydrous, which method comprises, reacting a fatty acid with a calcium salt, reactive with fatty acid to form a soap, but insufficient in amount to react with all of the fatty acid, then reacting, in situ, the uncombined fatty acid with a high boiling alcohol, whereby to provide a mass comprised of calcium salt of fatty acid mingled with a fatty acid ester having at least one free hydroxyl group.

3. The method which consists in substantially conjointly reacting a fatty acid with lime, insufficient in amount to react with all of the fatty acid, and with a high boiling alcohol adapted to esterify the remainder of the fatty acid, to provide a body consisting of the calcium salt of fatty acid mingled with a fatty acid ester having at least one free hydroxyl group.

4. The method which comprises, reacting lime with a quota of stearic acid in excess of the quota required to combine with the lime, then reacting the excess of fatty acid with a high boiling alcohol to provide, in the presence of the calcium salt of fatty acid, a fatty acid ester having free hydroxyl groups.

5. The method of making a base soluble in mineral oil to provide an anhydrous grease there-

from, which method comprises, forming a dry soap of a fatty acid in the presence of a quantity of fatty acid in excess of that required to form the soap and reacting the excess of fatty acid with an aliphatic alcohol which is reactive in respect thereto to form, in situ, a fatty acid ester having at least one free hydroxyl group.

6. A method of making a grease base which comprises, heating a mass of fatty acid partially saponified with lime with a polyhydric alcohol to esterify the saponified component of the fatty acid, to provide in the mass a quota of fatty acid ester having at least one free hydroxyl group, which is soluble in mineral oil and which possesses the capacity to dissolve the fatty acid component which is saponified.

7. The method of making an anhydrous grease base which comprises, forming a mass containing free fatty acid and fatty acid soap adapted to make a grease with mineral oil, and heating this mass with a quota of material reactive in respect to the free fatty acid, to provide a reaction component in the mass which has at least one free hydroxyl group and which is soluble in mineral oil and which is a solvent for the fatty acid soap.

8. A method of making an anhydrous grease base which consists in forming a fatty acid soap adapted to make a grease with mineral oil, and forming a partial ester of fatty acid which has at least one free hydroxyl group, in situ, during at least a portion of the time that the soap is being formed, the amount of ester formed being sufficient to solubilize the soap in mineral oil sufficient in quantity to make a grease therewith.

9. The method of making an anhydrous body soluble in mineral oil to form a grease therefrom, which method consists in saponifying a major portion of a body of fatty acid to form a substantially anhydrous fatty acid soap and in reacting the remaining minor portion of fatty acid with a body adapted to provide therefrom a reaction component which has at least one free hydroxyl group, which is soluble in mineral oil, which is a solvent for fatty acid soap and which is present in sufficient quantity to render all of the said soap soluble in mineral oil.

LATIMER D. MYERS.

#### CERTIFICATE OF CORRECTION.

Patent No. 2,151,641.

March 21, 1939.

LATIMER D. MYERS.

It is hereby certified that error appears in the printed specification of the above numbered patent requiring correction as follows: Page 3, second column, line 10, for "6%" read 6.9%; and that the said Letters Patent should be read with this correction therein that the same may conform to the record of the case in the Patent Office.

Signed and sealed this 18th day of April, A. D. 1939.

Henry Van Arsdale

(Seal)

Acting Commissioner of Patents